

## UNITED STATES PATENT OFFICE

LOUIS LENFANT, OF PARIS, FRANCE, ASSIGNOR TO CARTIER, SOCIETE ANONYME, OF PARIS, FRANCE, A COMPANY OF FRANCE

## GOLD ALLOY

No Drawing. Application filed July 18, 1931, Serial No. 551,793, and in France March 10, 1931.

The present invention has for its object a gold alloy which has the property of being softened by tempering and hardened by annealing at low temperature.

5 It comprises a certain amount of gold according to the fineness of the alloy that is desired.

The remainder consists of silver and copper, and a certain amount of chromium 10 and cobalt which must always be employed together according to the present invention.

The ratio of the amount of copper to the amount of silver will preferably average from 1.2 to 1.5 according to the desired shade of 15 the alloy.

The ratios of the quantities of chromium and cobalt to the whole alloy will be 0.5 to 4 per cent for the cobalt and 0.5 to 1 per cent for the chromium according to the hardening 20 effect that is to be obtained.

The hardness of the alloy immediately after casting is 168 Brinnell.

By way of example, I may indicate that for an alloy containing 75 per cent of gold, 25 13.5 per cent of copper, 10 per cent of silver, 1 per cent of cobalt, 0.5 per cent of chromium, tempering lowers said hardness to 140 and a heating at 200° C. for 4 hours brings it to 217.

For an alloy containing 65 per cent of gold, 30 19.5 per cent of copper, 14 per cent of silver, 1 per cent of cobalt, 0.5 per cent of chromium the hardness in the raw state is 174, after tempering 147 and after annealing 260.

These alloys never have any micro-fissurations. They are easily rolled in the cold state, are easily welded and their hardness makes it possible to give them a remarkable polish.

Said alloys are well adapted to the manufacture of jewels, boxes or plates either for domestic or for laboratory purposes. They are especially well suited to the manufacture 40 of gold cutlery.

The micrographic study of said alloys 45 shows a structure having a very fine grain, after tempering and annealing, which ensures a perfect homogeneity.

The advantages of said gold alloys are the following:

50 1. It is possible to harden the alloy at will,

which allows to shape an article while the metal is soft, and then to give it the required hardness after treatment by annealing. The low temperature at which said annealing takes place makes it possible to avoid any 55 injury of the article.

2. These alloys forge as well in the hot as in the cold state, which is generally not possible with ordinary gold alloys.

3. These alloys do not cause any alteration 60 in the shade of the enamels.

4. They can be given an especially high polish owing to the hardness that is imparted to them by annealing, which hardness is much greater than that of other commercial gold 65 alloys.

It should be well understood that the examples that have been indicated can be modified without departing from the spirit of the invention as comprehended within the scope 70 of the appended claims.

What I claim is:

1. An alloy containing:

|          | Per cent  |
|----------|-----------|
| Gold     | 75-65     |
| Copper   | 13.5-19.5 |
| Silver   | 10-14     |
| Cobalt   | 1         |
| Chromium | 0.5       |

in which the ratio of the percentage of copper to that of silver is comprised between 1.2 and 1.6.

2. An alloy containing: gold, 75 per cent, copper, 13.5 per cent, silver, 10 per cent, cobalt, 1 per cent and chromium, 0.5 per cent.

3. An alloy containing: gold, 65 per cent, copper, 19.5 per cent, silver, 14 per cent, cobalt 1 per cent and chromium 0.5 per cent.

In testimony whereof, I have signed the foregoing specification.

LOUIS LENFANT.

95

100